

G. E. BARTOL, JR.  
PROCESS OF MANUFACTURING PENS WITH ANGULAR NIBS.  
APPLICATION FILED DEC 31, 1921.

1,437,631.

Patented Dec. 5, 1922.



FIG. 1.



FIG. 2.



FIG. 3.



FIG. 4.

INVENTOR

WITNESS:

Bob. M. Kitchel.

George E. Bartol, Jr.  
BY  
Frank S. Russel  
ATTORNEY.

Patented Dec. 5, 1922.

1,437,631

# UNITED STATES PATENT OFFICE.

GEORGE E. BARTOL, JR., OF PHILADELPHIA, PENNSYLVANIA, ASSIGNOR TO C. HOWARD HUNT PEN COMPANY, OF CAMDEN, NEW JERSEY, A CORPORATION OF NEW JERSEY.

## PROCESS OF MANUFACTURING PENS WITH ANGULAR NIBS.

Application filed December 31, 1921. Serial No. 526,198.

*To all whom it may concern:*

Be it known that I, GEORGE E. BARTOL, Jr., a citizen of the United States, residing at Philadelphia, county of Philadelphia, 5 and State of Pennsylvania, have invented a new and useful Improvement in Processes of Manufacturing Pens with Angular Nibs, of which the following is a full, clear, and exact description, reference being had to 10 the accompanying drawings, which form a part of this specification.

In the manufacture of pens provided with wide, upwardly displaced, multiple nibbed extremities, such as are used in 15 drawing thick lines, as in printing show cards, the usual process results in a pen whose extremity is comparatively soft and which, while sufficiently flexible, is inelastic in that, when once bent or distorted 20 from its normal shape, it does not resume such shape, making its life quite ephemeral. Moreover, such a pen does not well resist the action of the ink. It is even quite difficult, by the usual process, to produce a 25 pen which is wholly undistorted, at the final stage of manufacture, because, after the upsetting of the extremity, the subsequent polishing or burnishing process tends to distort the nibs, and there is therefore con- 30 siderable loss in manufacture.

In the usual process, one or two slits are formed in the wide extremity, providing 35 two or three nibs. The temper of the pen is then drawn by heating to a moderate temperature followed by slow cooling. The extremity of the pen, while the pen is cold, is then upset in a press. These operations produce a pen which is comparatively soft and which, while more or less flexible, pos- 40 sesses little elasticity. Therefore, in the subsequent polishing or burnishing operation, any incidental distortion of the nibs is apt to be permanent; while even if a perfectly shaped product is turned out, the 45 comparative inelasticity of the bent extremity makes the life of the pen quite short.

In order that my improved process may be more readily understood, I have illustrated certain operations characterizing 50 such process in the accompanying drawings, in which—

Fig. 1 is a perspective view of an unfin- 55 ished pen as it appears before the upsetting operation.

Fig. 2 is a perspective view of the anvil

(the adjustable stops being omitted) with the pen positioned thereon, and of the heater and upsetting die.

Fig. 3 is a plan view of the anvil, the pen positioned thereon and the adjustable stops. 60

Fig. 4 is a perspective view of a finished pen.

The preliminary steps in the manufacture of the pen need not be described. It may be mentioned, however, that the pen *a* 65 is shaped to its final form, including the slitting of the extremity to form the multiple nib, except that the extremity of the nibs has not been bent back (see Fig. 1) and is then polished in a tumbling machine. 70

The pen is then placed on a rest, preferably an anvil *a*, as shown in Fig. 2. The front of the anvil slopes downward from the plane of the rest, as shown at *b*, at an angle thereto corresponding to the angle to 75 which the front extremity of the pen is to be bent. The operator places the pen on the rest and pushes it forward until it engages the adjustable stops *c*, *c* (Fig. 3) on opposite sides of the rest. In this position 80 the nibs of the pen overhang the front edge of the rest a distance corresponding to the desired length of the extremity to be upset.

A Bunsen blow-pipe *d* is positioned to direct a flame over the front edge of the anvil 85 and in a direction nearly or quite parallel to the inclined front face *b*. Above the front of the anvil is a hammer die *e* having an inclined lower face *f* extending parallel to the inclined front face *b* of the an- 90 vil and, back of that, a horizontally ex- tending face *g* adapted to engage that part of the pen immediately back of the extremity to be upset.

The flame of the blow pipe is constantly 95 playing across the space in front of the front edge of the pen-rest. When the pen is positioned on the anvil, its extremity quickly heats to a red heat. While the pen, on the line of bending, must be raised to 100 such heat, the flame may or may not play directly thereon, it being understood that, by conduction, the part of the pen immediately adjacent to the part enveloped in the flame will be highly heated. The upset- 105 ting die or punch is then moved down into contact with the front of the pen, thereby upsetting the extremity. The extremity is thus gripped between two metallic surfaces. The faces *f*, *g* of the die are cold, while the 110

opposing surfaces of the anvil are comparatively cold, as the flame does not play directly thereon. The engagement of the face *g* of the anvil with the pen just back of its 5 upset extremity, prevents tilting of the body of the pen or restores it to horizontal position of initially tilted. The die is retracted quite quickly after the upsetting operation. The shape of the complete pen is shown in 10 Fig. 4, *y* representing the upset extremity.

After the final shaping operation, the pen is polished or burnished.

The local application of high heat to that 15 part of the pen which is to be bent and the immediately following upsetting and chilling operation harden the point and impart to it such elasticity that the nibs, if distorted by ordinary pressure, resume their normal shape. The subsequent burnishing 20 operation does not, therefore, distort the nibs in the least degree, so that, at the final stage of manufacture, all the pens are perfectly shaped. In use, the pens are surprisingly durable, due to the temper being such 25 as to combine the desired qualities of hardness, flexibility and elasticity, and resist very well the corroding action of ink. This particular type of pen, as ordinarily manufactured, is especially deficient in these 30 qualities, and if distorting pressure be applied thereto, as is frequently the case in ordinary use, the nibs will spread and fail to resume their normal shape, thus virtually ruining the pen. It will be understood, 35 therefore, why my improved process effects a substantial advance in the art.

While my invention has been shown and described as applied to pens with wide three-nibbed points, it is also applicable to pens 40 with sharp two-nibbed points the extremities of which are displaced angularly to the body of the pen.

Having now fully described my invention, what I claim and desire to protect by Letters Patent is:—

1. In the process of making pens, with upwardly displaced extremities, the steps

which comprise taking a pen slotted and shaped except for the upsetting of the extremity, heating the extremity to a red heat 50 and simultaneously upsetting and chilling the end, thereby producing a comparatively hard and elastic extremity.

2. In the process of making pens, with upwardly displaced extremities, the steps 55 which comprise taking a pen slotted and shaped except for the upsetting of the extremity, placing only the extremity of the pen in a highly heated zone adapted to suddenly elevate such extremity to a temperature corresponding to a red heat, upsetting the end while it is being subjected to such heat and immediately chilling the pen.

3. In the process of making pens, with upwardly displaced extremities, the steps 65 which comprise taking a pen slotted and shaped except for the upsetting of the extremity, placing only the extremity of the pen in a highly heated zone adapted to suddenly elevate such extremity to a temperature corresponding to a red heat, and 70 immediately confining the extremity between two metallic surfaces, one at least of which is relatively cold, extending at an angle to the direction of extension of the 75 body of the pen, thereby simultaneously upsetting and chilling said extremity.

4. In the process of making pens, with upwardly displaced extremities, the steps which comprise taking a pen slotted and shaped 80 except for the upsetting of the extremity, laying the pen on a relatively cold anvil in such position as to leave the extremity to be upset projecting beyond the anvil, directly heating the projecting extremity only 85 of the pen quickly to a red heat, and immediately upsetting the highly heated projecting extremity by means of a cold punch die.

In testimony of which invention, I have 90 hereunto set my hand, at Philadelphia, Penn., on this 30th day of December, 1921.

GEORGE E. BARTOL, JR.